

J. T. TERRY, JR.  
PROCESS FOR THE CONCENTRATION OF ORE.  
APPLICATION FILED MAR. 24, 1917.

1,254,173.

Patented Jan. 22, 1918.



Attest.  
Charles C. Becker.

Inventor.  
Joseph T. Terry, Jr.,  
Los Angeles, California.  
His Attorneys

# UNITED STATES PATENT OFFICE.

JOSEPH T. TERRY, JR., OF MASCOT, TENNESSEE.

## PROCESS FOR THE CONCENTRATION OF ORE.

1,254,173.

Specification of Letters Patent. Patented Jan. 22, 1918.

Application filed March 24, 1917. Serial No. 157,188.

*To all whom it may concern:*

Be it known that I, JOSEPH T. TERRY, Jr., a citizen of the United States of America, residing at Mascot, in the county of Knox, 5 State of Tennessee, have invented certain new and useful Improvements in Processes for the Concentration of Ore, of which the following is a specification.

This invention relates primarily to processes of extracting and recovering the metallic elements of finely crushed ore by means of the combined action of certain chemicals and novel mechanical devices, and has for its prime object the simplification of existing 10 methods for the separation of metallic sulfids, as for example the sulfids of zinc, lead, copper and metallic copper, or any combination thereof, from iron sulfids and gangue, and the attainment of an unusually high percentage of metal recovery.

A further object of the invention is to afford a process so economical and efficacious as to render profitable the treatment of ores of low grade and peculiar composition 15 which have heretofore been practically neglected as a source of supply.

Other objects and advantages will become apparent upon consideration of the following portions of the specification and the appended claims:

In the accompanying drawing, wherein like numerals refer to like parts throughout, the figure is a sectional elevation depicting the preferred apparatus evolved by me for 20 carrying out the process.

Referring to said figure, 1 denotes a common type of ball-mill in which the rough ore collected from hopper 2 by scoop 3 is finely crushed in the presence of water and shall 25 hereinafter be termed the "pulp." Being ejected from funnel 4 the pulp is conducted by a launder 5 to the top of pipe 6 and thence successively into stationary air-tight drums 7 and 8 which are closed above, connected by pipes 9 and 10, and contain paddles 11 and 12 fixed upon revolving shafts 13 and 14 driven by means of pulleys 15 and belts 16.

Disposed above pipes 6 and 10 are small 30 tanks 17 and 18 provided with depending spouts 19 and 20 discharging into said pipes. Passing from drum 8 the pulp is conveyed by pipe 21 to a cylindrical chamber 22 which communicates with a tube 23 extending upward and rebent over the edge of a spitzkasten 24, the latter being provided with a

baffle-plate 25 disposed opposite the mouth of said tube and a drain 26.

Projecting within chamber 22 is a pressure-fluid supply-pipe 27 which is inclosed 60 and serves to support a closely wound helical spring 28 terminating in a solid cap 29, and it will be appreciated that air or other gas being forced through pipe 27 will escape through the interstices of said spring and 65 thus be thoroughly disseminated throughout the mixture present in said chamber.

Having thus pointed out the construction and function of the preferred form of apparatus, as illustrated, the process involved 70 may be described as follows:—Tank 17 having been filled with a solution of ammonia hydroxid or with a solution containing or capable of liberating ammonia, such as ammoniacal liquor by-product in the manufacture 75 of illuminating gas, and tank 18 with a suitable oleaginous modifying reagent, such as pine oil or a solution of metallic oleates resulting from the combination and saponification of metallic oxides and salts with hydrocarbons of the olefin series, as for example 80 aluminum salts combined with olefin oils of mineral origin, the mill 1 is then set in motion and the pulp flowing into pipe 6 is there mingled with the ammoniacal solution 85 discharged from spout 19. Reaching the interior of drum 7 the mixture is thoroughly agitated and the ingredients thereof intimately combined by the action of paddle 11, flowing thence through pipes 9 and 10 into 90 drum 8, together with the oil or other modifying reagent supplied by tank 18, where it is subjected to a further vigorous agitation through the agency of paddle 12 and the ingredients thus more perfectly combined. 95

From drum 8 the mixture is next conveyed by pipe 21 to chamber 22 and passing upward therein is thoroughly aerated by means of the gas forced from pipe 27 through the interstices of spring 28, the gas 100 thus injected serving to convert the mixture into a froth or mass of small bubbles. The froth thus created is carried upward and discharged from tube 23 into spitzkasten 24 behind the baffle-plate 25, and passing thereunder rises to the water level and flows off over the forward edge of the tank substantially in the manner depicted.

The innumerable oil-filmed bubbles 105 composing the froth referred to have the property of attracting, enmeshing and retaining in suspension the fine particles of metal

present in the pulp aforesaid, and one of the most important features of this process resides in my discovery that ammonia in solution has the effect of oxidizing the iron sulfids sufficiently to destroy the affinity which would otherwise exist between such sulfids and the oil or other modifying reagent employed, and being a solvent for the oxids of lead, zinc and copper it has the effect of 5 cleansing their sulfid particles and thus decidedly increases their affinity for said reagent: the result being that the particles of iron and gangue gravitate to the bottom of the spitzkasten and the percentage of valuable metals recovered is rendered unusually 10 high.

A further important feature of this process lies in the fact, above stated, that drums 7 and 8 are air-tight, for I have discovered 20 that a greater recovery of metallic sulfids is attained by mixing the pulp and the modifying reagents in a vessel from which air or other gas is excluded, as it has been determined that the presence of the latter during 25 the operation in question serves to obstruct that intimate combination of the ore particles with the reagents which is sought to be achieved and upon which the success of this or any similar process must largely depend.

30 It should further be observed that I have found it advantageous to treat the crushed ore, preferably while in the mill, with a solution of calcium hydroxid and sodium thiosulfate, as the lime neutralizes such acid 35 or acid salts as may be present in the ore, while the alkaline thiosulfate cleanses the metallic sulfids by dissolving oxids and other soluble metallic constituents, and thus permits the use of less ammonia than would 40 otherwise be necessary in the process.

Finally it should be noted that I do not intend to restrict this invention to the introduction of ammonia in advance of the introduction of the oil or other modifying 45 reagent employed, but may add such a reagent simultaneously and in combination with the ammonia in the form of an emulsion or soap.

Having thus fully described the process 50 and the preferred means for carrying it out, what I claim as new and desire to secure by Letters-Patent is:—

1. The method of recovering the valuable elements of complex sulfid ore containing 55 iron sulfids, which comprises the treatment of crushed ore with an ammoniacal solution, thereby altering the iron sulfids to render the same substantially immune to flotation, and creating in the mixture uprising bubbles 60 carrying the metallic values.

2. The method of recovering the valuable elements of complex sulfid ore containing iron sulfids, which comprises the treatment of crushed ore with an ammoniacal solution 65 and a frothing agent, thereby altering the

iron sulfids to render the same substantially immune to flotation, and creating in the mixture uprising bubbles carrying the metallic values.

3. The method of recovering the valuable 70 elements of complex sulfid ore containing iron sulfids, which comprises the treatment of crushed ore with a solution of lime and an ammoniacal solution, thereby altering the iron sulfids to render the same substantially 75 immune to flotation, and creating in the mixture uprising bubbles carrying the metallic values.

4. The method of recovering the valuable 80 elements of complex sulfid ore containing iron sulfids, which comprises the treatment of crushed ore with a solution of sodium thiosulfate and an ammoniacal solution, thereby altering the iron sulfids to render the same substantially immune to flotation, 85 and creating in the mixture uprising bubbles carrying the metallic values.

5. The method of recovering the valuable 90 elements of complex sulfid ore containing iron sulfids, which comprises the treatment of crushed ore with a solution of lime, an ammoniacal solution and a frothing agent, thereby altering the iron sulfids to render the same substantially immune to flotation, 95 and creating in the mixture uprising bubbles carrying the metallic values.

6. The method of recovering the valuable 100 elements of complex sulfid ore containing iron sulfids, which comprises the treatment of crushed ore with a solution of sodium thiosulfate, an ammoniacal solution, and a frothing agent, thereby altering the iron sulfids to render the same substantially immune to flotation, and creating in the mixture uprising bubbles 105 carrying the metallic values.

7. The method of recovering the valuable 110 elements of complex sulfid ore containing iron sulfids, which comprises the treatment of crushed ore with a solution of lime and sodium thiosulfate, and an ammoniacal solution, thereby altering the iron sulfids to render the same substantially immune to flotation, and creating in the mixture uprising bubbles carrying the metallic values. 115

8. The method of recovering the valuable 120 elements of complex sulfid ore containing iron sulfids, which comprises the treatment of crushed ore with a solution of lime and sodium thiosulfate, a frothing agent, and an ammoniacal solution, thereby altering the iron sulfids to render the same substantially immune to flotation, and creating in the mixture uprising bubbles carrying the metallic values. 125

9. The method of recovering the valuable 130 elements of complex sulfid ore containing iron sulfids, which comprises the treatment of crushed ore with an ammoniacal solution, thereby altering the iron sulfids to render

the same substantially immune to flotation, and subsequently creating in the mixture uprising bubbles carrying the metallic values.

10. The method of recovering the valuable elements of complex sulfid ore containing iron sulfids, which comprises the treatment of crushed ore with an ammoniacal solution and a frothing agent, thereby altering the iron sulfids to render the same substantially immune to flotation, and subsequently creating in the mixture uprising bubbles carrying the metallic values.

11. The method of recovering the valuable elements of complex sulfid ore containing iron sulfids, which comprises the treatment of crushed ore with a solution of lime and an ammoniacal solution, thereby altering the iron sulfids to render the same substantially immune to flotation, and subsequently creating in the mixture uprising bubbles carrying the metallic values.

12. The method of recovering the valuable elements of complex sulfid ore containing iron sulfids, which comprises the treatment of crushed ore with a solution of sodium thiosulfate and an ammoniacal solution, thereby altering the iron sulfids to render the same substantially immune to flotation, and subsequently creating in the mixture 25 uprising bubbles carrying the metallic values.

30

30 13. The method of recovering the valuable elements of complex sulfid ore containing iron sulfids, which comprises the treatment of crushed ore with a solution of lime,  
35 an ammoniacal solution, and a frothing agent, thereby altering the iron sulfids to render the same substantially immune to flotation, and subsequently creating in the mixture uprising bubbles carrying the metallic values.

40. The method of recovering the valuable elements of complex sulfid ore containing iron sulfids, which comprises the treatment of crushed ore with a solution of sodium thiosulfate, an ammoniacal solution, and a frothing agent, thereby altering the iron sulfids to render the same substantially immune to flotation, and subsequently creating in the mixture uprising bubbles carrying the metallic values.

50 ing the metallic values.  
15. The method of recovering the valuable elements of complex sulfid ore containing iron sulfids, which comprises the treatment of crushed ore with a solution of lime  
55 and sodium thiosulfate, and an ammoniacal solution, thereby altering the iron sulfids to render the same substantially immune to flotation, and subsequently creating in the mixture uprising bubbles carrying the metallic values.

60 traffic varieties.  
16. The method of recovering the valuable elements of complex sulfid ore containing iron sulfids, which comprises the treatment of crushed ore with a solution of lime  
65 and sodium thiosulfate, a frothing agent,

and an ammoniacal solution, thereby altering the iron sulfids to render the same substantially immune to flotation, and subsequently creating in the mixture uprising bubbles carrying the metallic values.

17. The method of recovering the valuable elements of complex sulfid ore containing iron sulfids, which comprises the treatment of crushed ore with an ammoniacal solution, thereby altering the iron sulfids to render the same substantially immune to flotation, agitating the mixture substantially out of contact with air, and subsequently creating in the mixture uprising bubbles carrying the metallic values. 75 80

18. The method of recovering the valuable elements of complex sulfid ore containing iron sulfids, which comprises the treatment of crushed ore with an ammoniacal solution, and a frothing agent, thereby altering the iron sulfids to render the same substantially immune to flotation, agitating the mixture substantially out of contact with air, and subsequently creating in the mixture uprising bubbles carrying the metallic values.

19. The method of recovering the valuable elements of complex sulfid ore containing iron sulfids, which comprises the treatment of crushed ore with a solution of lime and an ammoniacal solution, thereby altering the iron sulfids to render the same substantially immune to flotation, agitating the mixture substantially out of contact with air, and subsequently creating in the mixture uprising bubbles carrying the metallic values. 95 100

20. The method of recovering the valuable elements of complex sulfid ore containing iron sulfids, which comprises the treatment of crushed ore with a solution of sodium thiosulfate and an ammoniacal solution, thereby altering the iron sulfids to render the same substantially immune to flotation, agitating the mixture substantially out of contact with air, and subsequently creating in the mixture uprising bubbles carrying the metallic values. 105 110

21. The method of recovering the valuable elements of complex sulfid ore containing iron sulfids, which comprises the treatment of crushed ore with a solution of lime, an ammoniacal solution, and a frothing agent, thereby altering the iron sulfids to render the same substantially immune to flotation, agitating the mixture substantially out of contact with air, and subsequently creating in the mixture uprising bubbles carrying the metallic values. 115 120

22. The method of recovering the valuable elements of complex sulfid ore containing iron sulfids, which comprises the treatment of crushed ore with a solution of sodium thiosulfate, an ammoniacal solution, and a frothing agent, thereby altering the 130

iron sulfids to render the same substantially immune to flotation, agitating the mixture substantially out of contact with air, and subsequently creating in the mixture up-  
5 rising bubbles carrying the metallic values.

23. The method of recovering the valuable elements of complex sulfid ore containing iron sulfids, which comprises the treatment of crushed ore with a solution of lime and 10 sodium thiosulfate, and an ammoniacal solution, thereby altering the iron sulfids to render the same substantially immune to flotation, agitating the mixture substantially out of contact with air, and subsequently creating in the mixture up-  
15 rising bubbles carrying the metallic values.

24. The method of recovering the valuable elements of complex sulfid ore containing iron sulfids, which comprises the treatment of crushed ore with a solution of lime and sodium thiosulfate, a frothing agent, and an ammoniacal solution, thereby 20 altering the iron sulfids to render the same substantially immune to flotation, agitating the mixture substantially out of contact 25 with air, and subsequently creating in the mixture uprisng bubbles carrying the metallic values.

JOSEPH T. TERRY, JR.

Witnesses:

HARRY L. LAWSON,  
M. R. BARTON.